

## UNITED STATES PATENT OFFICE

2,233,576

STIFFENING MEMBER FOR SHOES AND THE  
LIKE

Paul A. Balon, Arlington, N. J., and Harold S. Holt, Wilmington, Del., assignors to The Celsastic Corporation, Wilmington, Del., a corporation of Delaware

No Drawing. Application February 4, 1939,  
Serial No. 254,604

10 Claims. (CL 36—77)

This invention relates to stiffening members for shoes and the like and, more particularly, to box toes and counters made from a web of fibrous material impregnated with a thermoplastic substance.

Material for stiffening members is commonly made by impregnating a suitable fabric with a thermoplastic composition. Blanks of suitable size and shape cut from the impregnated goods, usually skived to a tapered edge, are shaped into conformity with the shoe last by being softened by heat and, while still soft, stretched in place over the last. Stiffening material of this type is designated as heat-softening, to distinguish it from those which are softened for lasting by being moistened with solvent or with water and which are designated as solvent-softening and water-softening, respectively.

Heat-softening stiffening members are ordinarily softened for lasting by being placed on a so-called "steamer", i. e., a box or tray with a perforated bottom set over a bath of boiling water. It is, accordingly, necessary that a heat-softening stiffening material shall become effectively softened at the ordinary temperature of this device, which will range between about 80° and 100° C., and it is further essential that the blank shall then retain its softness during the brief period, amounting ordinarily to from 10 to 15 seconds, which is required for completing the operation of the pulling-over machine. At the same time, it is essential that the box toe or counter, as a part of the structure of the finished shoe, shall not be subject to deformation by heat in the course of ordinary and prolonged wearing, or of storage and display.

It is further desirable that stiffening members used in the construction of ordinary dress shoes, as differentiated from work shoes having the so-called "safety toe" feature, shall have adequate rigidity and toughness without being excessively thick which would impair the appearance of the shoe as a whole. Further requirements are that the material shall not be subject to deterioration with age, and that it shall at no time either in

the course of the construction of the shoe or during its subsequent service, cause stain or other damage to the leather or fabric with which it is associated in the shoe, and also that it be not subject to damage either by immersion of the shoe in water or by protracted contact with moisture or with perspiration from the feet of the wearer.

It is an object of the present invention to provide improved stiffening material of the heat-softening type. More specifically, it is an object of the invention to provide such a material presenting a combination of desirable properties not heretofore associated with stiffening materials of the impregnated heat-softening type, namely, a material which is softened adequately by the temperature of the steamer and retains its softness during the subsequent ordinary operation of lasting, which is satisfactorily form-stable, i. e., is free from deformation by heat at temperatures of ordinary service, storage and display, which, in a thickness acceptable for dress shoes, has notable strength and toughness and rigidity, which does not strain or otherwise damage adjacent materials in the shoe, and which is not subject to deterioration with age nor to softening or deterioration by immersion in water or by prolonged exposure to warmth and moisture in service. Other objects of the invention will be apparent from the description given hereinafter.

The above objects are accomplished according to the present invention by the use, as a stiffening member for shoes and the like, of a web of fibrous material such as flannel, felt, paper, and similar fibrous material, impregnated with a composition comprising essentially beta-naphthol-modified rubber, of beta-naphthol content between 10-30%, by weight, and a compatible auxiliary component, the composition having a temperature of plasticity of 70-90° C. and a softening point of 75-100° C.

The term "temperature of plasticity" is used herein to denote that temperature at which in the A. S. T. M. ring-and-ball test (D36-26, A. S. T. M. Standards, 1927, II, 496), the ball starts to sink into the heated impregnant being tested. It

has been determined that this temperature substantially coincides with the lowest temperature at which the usual stiffener impregnated with the impregnant in question is softened sufficiently to be lasted. In ordinary practice, the temperature of plasticity should not be higher than the temperature of the steamer, i. e., between 80-100° C., and, preferably, between 70-90° C. The term "softening point" is used herein to denote the temperature of the impregnant determined as the softening point in accordance with the A. S. T. M. ring-and-ball test (D36-26, A. S. T. M. Standards, 1927, II, 496), i. e., the temperature of the impregnant at the moment when the sinking ball arrives at the bottom of the test container.

The beta-naphthol-modified rubber, which may be produced in accordance with the method set forth in United States Patent 2,158,530 to Ira Williams and entitled "Thermoplastic derivatives of rubber," may be graded in accordance with the proportion of beta-naphthol with which the rubber has been brought into reaction. It is believed that not necessarily all of the beta-naphthol is actually chemically combined with the rubber but any amount in excess of that which is actually chemically combined, nevertheless remains closely associated with the rubber and has the effect of modifying its properties.

The naphthol-modified rubbers contemplated for use in the present invention are those in which the beta-naphthol content ranges between 10-30%, by weight, a beta-naphthol content of 20% being preferred. The term "beta-naphthol-modified rubber" is used hereinafter throughout the specification and claims to denote the beta-naphthol-modified rubber such as may be obtained by the process disclosed and claimed in said United States Patent 2,158,530, and which has a beta-naphthol content between 10-30%, by weight. It has been found that naphthol-modified rubbers outside this range are not adapted for the purposes of the present invention.

Beta-naphthol-modified rubber possesses remarkable toughness and strength. At ordinary temperatures it is rigid rather than "rubbery," resembling hard rubber (ebonite) but differs therefrom in being capable of being melted without serious decomposition. The high softening point and the high viscosity of this material in molten condition precludes the use of beta-naphthol-modified rubber by itself as an impregnant for shoe stiffening materials since it does not become mobile enough at practical temperatures to permit acceptable impregnation of fibrous material by ordinarily available methods.

It has now been discovered that auxiliary ingredients may be combined with beta-naphthol-modified rubber to give a composition highly advantageous as an impregnant for shoe stiffening, that is, by combining the beta-naphthol-modified rubber with auxiliary ingredients a composition is obtained with a softening point and a temperature of plasticity within a convenient range and that gives a melt of suitably low viscosity for impregnation by ordinary methods and, yet, retains the toughness and strength of the beta-naphthol-modified rubber and gives an impregnated web of acceptable form-stability. In addition, the cost of impregnant compares most favorably with the cost of impregnants heretofore used.

The auxiliary component of the impregnant according to the present invention should give a resulting composition with the beta-naphthol-

modified rubber that will have a temperature of plasticity between 70-90° C. and a softening temperature of 75-100° C. The auxiliary component may be composed of one or several auxiliary ingredients conveniently classified as plasticizers, 5 modifiers, and extenders.

Plasticizers for beta-naphthol-modified rubber may be defined as substances which are compatible with the beta-naphthol-modified rubber and can be incorporated homogeneously with it 10 by being melted together with it, without the assistance of a solvent, and which have the effects of lowering the softening point of the beta-naphthol-modified rubber and the viscosity of the melt, of decreasing the temperature of 15 plasticity without unduly decreasing the form-stability, and of improving the toughness and, particularly, the flexibility.

Modifiers for beta-naphthol-modified rubber may be defined as substances which have the 20 same general effects as the plasticizers but a much more marked effect upon the form-stability which necessitates limiting their proportion in the mix to a lower percentage than is necessary with the plasticizers. 25

Extenders may be defined as substances characterized by being compatible with beta-naphthol-modified rubber and by being fusible therewith to a homogeneous mixture but by being without beneficial effect upon the toughness and 30 flexibility of the beta-naphthol-modified rubber and, in fact, tending to impair these properties somewhat. The extenders do not substantially alter the form-stability of the mixture and some 35 are without substantial influence on the softening point and the temperature of plasticity while others tend to lower these to some extent.

The proportion of auxiliary component to be used in the impregnant must give a composition having a temperature of plasticity between 40 70-90° C. and a softening point between 75-100° C. because, with respect to the temperature of plasticity, there is the practical necessity of adequate softening of the impregnated shoe stiffener at steamer temperatures while, with respect to the softening point, it has been found that compositions within the scope of the invention, having softening points not lower than about 75° C. will have satisfactory form-stability at temperatures of service while those of softening point not over about 100° C. can be melted to a suitably mobile liquid without the need of exceeding the temperature, around 190° C., at which they are safe from decomposition.

Since the effect of individual auxiliary ingredients on the beta-naphthol-modified rubber varies, it is not possible to define except within approximate operative limits the proportions of plasticizers, modifiers, and extenders, generically considered. However, in the light of the discussion given hereinafter, together with the numerous examples, those skilled in the art will be able to formulate readily preferred specific impregnant compositions within the scope of the invention. 65

In the following examples illustrating specific impregnant compositions according to the invention, and throughout the specification, all proportions are given by weight unless otherwise stated. The examples are grouped in tables as 70 follows:

Table I, Examples 1 to 13—use of plasticizer as sole auxiliary ingredient;

Table II, Examples 14 to 28—use of montan wax (either a plasticizer or an extender depend- 75

ing upon the proportion used) and another plasticizer together;

Table III, Examples 29 to 39—use of modifier as sole auxiliary ingredient;

5 Table IV, Examples 40 to 46—use of extenders only;

Table V, Examples 47 to 75—use of plasticizer and extender together;

10 Table VI, Example 76—use of plasticizer and modifier together; Example 77—use of plasticizer, modifier, and extender together.

Table I

|    | Example No.                     |     |     |     |     |     |     |
|----|---------------------------------|-----|-----|-----|-----|-----|-----|
|    | 1                               | 2   | 3   | 4   | 5   | 6   | 7   |
| 20 | Naphthol-modified rubber:       |     |     |     |     |     |     |
|    | Beta-naphthol, 10%              |     |     |     |     |     |     |
|    | 100                             | 100 | 100 | 100 | 100 | 100 | 100 |
|    | Beta-naphthol, 20%              |     |     |     |     |     |     |
|    | 33                              | 43  | 67  | 82  | 100 |     |     |
|    | Beta-naphthol, 30%              |     |     |     |     |     |     |
|    | 25                              |     |     |     |     |     |     |
|    | "Cumar" A.X.                    |     |     |     |     |     |     |
|    | Montan wax                      |     |     |     |     |     |     |
|    | Temperature of plasticity (°C.) | 83  | 81  | 79  | 84  | 83  | 84  |
| 25 | Softening point (°C.)           | 96  | 103 | 99  | 98  | 95  | 91  |

|    | Example No.                     |     |     |     |    |    |    |
|----|---------------------------------|-----|-----|-----|----|----|----|
|    | 8                               | 9   | 10  | 11  | 12 | 13 |    |
| 30 | Naphthol-modified rubber:       |     |     |     |    |    |    |
|    | Beta-naphthol, 10%              |     |     |     |    |    |    |
|    | 100                             | 100 | 100 | 100 |    |    |    |
|    | Beta-naphthol, 20%              |     |     |     |    |    |    |
|    | 33                              | 100 |     | 100 |    |    |    |
|    | Beta-naphthol, 30%              |     |     |     |    |    |    |
|    | 100                             |     |     |     |    |    |    |
|    | "Cumar" BX                      |     |     |     |    |    |    |
|    | Montan wax                      |     |     |     |    |    |    |
|    | Temperature of plasticity (°C.) | 73  | 81  | 78  | 85 | 80 | 85 |
|    | Softening point (°C.)           | 94  | 100 | 93  | 87 | 96 | 86 |

| 40 | Example No.                     |     |     |     |     |     |     |
|----|---------------------------------|-----|-----|-----|-----|-----|-----|
|    | 8                               | 9   | 10  | 11  | 12  | 13  | 14  |
|    | Naphthol-modified rubber:       |     |     |     |     |     |     |
|    | Beta-naphthol, 10%              |     |     |     |     |     |     |
|    | 100                             | 100 | 100 | 100 | 100 | 100 | 100 |
|    | Beta-naphthol, 20%              |     |     |     |     |     |     |
|    | 33                              | 100 |     | 100 |     |     |     |
|    | Beta-naphthol, 30%              |     |     |     |     |     |     |
|    | 100                             |     |     |     |     |     |     |
|    | "Cumar" BX                      |     |     |     |     |     |     |
|    | Montan wax                      |     |     |     |     |     |     |
|    | Temperature of plasticity (°C.) | 73  | 81  | 78  | 85  | 80  | 85  |
|    | Softening point (°C.)           | 94  | 100 | 93  | 87  | 96  | 86  |

Table II

|    | Example No.                     |     |     |     |     |     |     |
|----|---------------------------------|-----|-----|-----|-----|-----|-----|
|    | 14                              | 15  | 16  | 17  | 18  | 19  | 20  |
| 45 | Naphthol-modified rubber:       |     |     |     |     |     |     |
|    | Beta-naphthol, 10%              |     |     |     |     |     |     |
|    | 100                             | 100 | 100 | 100 | 100 | 100 | 100 |
|    | Beta-naphthol, 20%              |     |     |     |     |     |     |
|    | 33                              | 100 |     | 100 |     |     |     |
|    | Beta-naphthol, 30%              |     |     |     |     |     |     |
|    | 18                              | 20  |     | 22  |     | 100 | 25  |
|    | "Cumar" BX                      |     |     |     |     |     |     |
|    | "Neville X-1"                   |     |     |     |     |     |     |
|    | Montan wax                      |     |     |     |     |     |     |
| 55 | Temperature of plasticity (°C.) | 63  | 80  | 66  | 66  | 100 | 100 |
|    | Softening point (°C.)           | 84  | 82  | 82  | 83  | 85  | 80  |

| 60 | Example No.                     |     |     |     |     |     |     |
|----|---------------------------------|-----|-----|-----|-----|-----|-----|
|    | 14                              | 15  | 16  | 17  | 18  | 19  | 20  |
|    | Naphthol-modified rubber:       |     |     |     |     |     |     |
|    | Beta-naphthol, 10%              |     |     |     |     |     |     |
|    | 100                             | 100 | 100 | 100 | 100 | 100 | 100 |
|    | Beta-naphthol, 20%              |     |     |     |     |     |     |
|    | 33                              | 100 |     | 100 |     |     |     |
|    | Beta-naphthol, 30%              |     |     |     |     |     |     |
|    | 18                              | 20  |     | 22  |     | 100 | 25  |
|    | "Cumar" BX                      |     |     |     |     |     |     |
|    | "Neville X-1"                   |     |     |     |     |     |     |
|    | Montan wax                      |     |     |     |     |     |     |
|    | Temperature of plasticity (°C.) | 63  | 80  | 66  | 66  | 100 | 100 |
|    | Softening point (°C.)           | 84  | 82  | 82  | 83  | 85  | 80  |

Table II.—Continued

|  | Example No.                     |     |     |     |     |     |     |
|--|---------------------------------|-----|-----|-----|-----|-----|-----|
|  | 22                              | 23  | 24  | 25  | 26  | 27  | 28  |
|  | Naphthol-modified rubber:       |     |     |     |     |     |     |
|  | Beta-naphthol, 10%              |     |     |     |     |     |     |
|  | 100                             | 100 | 100 | 100 | 100 | 100 | 100 |
|  | Beta-naphthol, 20%              |     |     |     |     |     |     |
|  | 23                              | 100 | 100 | 18  | 100 |     |     |
|  | Beta-naphthol, 30%              |     |     |     |     |     |     |
|  | "Cumar" A.X.                    |     |     |     |     |     |     |
|  | "Neville X-1"                   |     |     |     |     |     |     |
|  | Montan wax                      |     |     |     |     |     |     |
|  | Temperature of plasticity (°C.) | 83  | 83  | 85  | 87  | 85  | 82  |
|  | Softening point (°C.)           | 86  | 83  | 86  | 93  | 86  | 83  |

Table III

|  | Example No.                     |     |     |     |     |     |
|--|---------------------------------|-----|-----|-----|-----|-----|
|  | 29                              | 30  | 31  | 32  | 33  | 34  |
|  | Naphthol-modified rubber:       |     |     |     |     |     |
|  | Beta-naphthol, 10%              |     |     |     |     |     |
|  | 100                             | 100 | 100 | 100 | 100 | 100 |
|  | Beta-naphthol, 20%              |     |     |     |     |     |
|  | 11                              | 13  |     |     |     |     |
|  | Beta-naphthol, 30%              |     |     |     |     |     |
|  | Paraffin wax                    |     |     |     |     |     |
|  | Ceresin wax                     |     |     |     |     |     |
|  | Japan wax                       |     |     |     |     |     |
|  | Temperature of plasticity (°C.) | 85  | 84  | 72  | 79  | 84  |
|  | Softening point (°C.)           | 104 | 108 | 109 | 103 | 104 |

|  | Example No.                     |     |     |     |     |     |
|--|---------------------------------|-----|-----|-----|-----|-----|
|  | 35                              | 36  | 37  | 38  | 39  |     |
|  | Naphthol-modified rubber:       |     |     |     |     |     |
|  | Beta-naphthol, 10%              |     |     |     |     |     |
|  | 100                             | 100 | 100 | 100 | 100 | 100 |
|  | Beta-naphthol, 20%              |     |     |     |     |     |
|  | 18                              | 11  | 18  | 13  | 18  |     |
|  | Beta-naphthol, 30%              |     |     |     |     |     |
|  | Paraffin wax                    |     |     |     |     |     |
|  | Gum resin                       |     |     |     |     |     |
|  | Limed resin (195° F.)           |     |     |     |     |     |
|  | Montan wax                      |     |     |     |     |     |
|  | Temperature of plasticity (°C.) | 86  | 80  | 79  | 84  | 83  |
|  | Softening point (°C.)           | 100 | 96  | 95  | 85  | 93  |

|  | Example No.                     |     |     |     |     |     |     |
|--|---------------------------------|-----|-----|-----|-----|-----|-----|
|  | 40                              | 41  | 42  | 43  | 44  | 45  | 46  |
|  | Naphthol-modified rubber:       |     |     |     |     |     |     |
|  | Beta-naphthol, 10%              |     |     |     |     |     |     |
|  | 100                             | 100 | 100 | 100 | 100 | 100 | 100 |
|  | Beta-naphthol, 20%              |     |     |     |     |     |     |
|  | 350                             |     |     |     |     |     |     |
|  | Beta-naphthol, 30%              |     |     |     |     |     |     |
|  | FF wood rosin                   |     |     |     |     |     |     |
|  | G gum resin                     |     |     |     |     |     |     |
|  | Limed resin (195° F.)           |     |     |     |     |     |     |
|  | Montan wax                      |     |     |     |     |     |     |
|  | Temperature of plasticity (°C.) | 87  | 80  | 79  | 84  | 83  | 85  |
|  | Softening point (°C.)           | 100 | 96  | 95  | 85  | 93  | 86  |

|  | Example No.                     |     |     |     |     |     |     |     |     |     |
|--|---------------------------------|-----|-----|-----|-----|-----|-----|-----|-----|-----|
|  | 47                              | 48  | 49  | 50  | 51  | 52  | 53  | 54  | 55  | 56  |
|  | Naphthol-modified rubber:       |     |     |     |     |     |     |     |     |     |
|  | Beta-naphthol, 10%              |     |     |     |     |     |     |     |     |     |
|  | 100                             | 100 | 100 | 100 | 100 | 100 | 100 | 100 | 100 | 100 |
|  | Beta-naphthol, 20%              |     |     |     |     |     |     |     |     |     |
|  | 25                              |     |     |     |     |     |     |     |     |     |
|  | Beta-naphthol, 30%              |     |     |     |     |     |     |     |     |     |
|  | "Cumar" A.X.                    |     |     |     |     |     |     |     |     |     |
|  | "Cumar" BX                      |     |     |     |     |     |     |     |     |     |
|  | "Neville X-1"                   |     |     |     |     |     |     |     |     |     |
|  | FF wood rosin                   |     |     |     |     |     |     |     |     |     |
|  | G gum resin                     |     |     |     |     |     |     |     |     |     |
|  | "Cumar" FX                      |     |     |     |     |     |     |     |     |     |
|  | Temperature of plasticity (°C.) | 87  | 77  | 83  | 85  | 69  | 69  | 70  | 71  | 78  |
|  | Softening point (°C.)           | 99  | 95  | 97  | 98  | 80  | 79  | 81  | 81  | 87  |

Table V.—Continued

| 5                                | Example No. |     |     |     |     |     |     |     |     |     | 8   |
|----------------------------------|-------------|-----|-----|-----|-----|-----|-----|-----|-----|-----|-----|
|                                  | 57          | 58  | 59  | 60  | 61  | 62  | 63  | 64  | 65  | 66  |     |
| <b>Naphthol-modified rubber:</b> |             |     |     |     |     |     |     |     |     |     |     |
| Beta-naphthol, 10%               |             |     |     |     |     |     |     |     |     |     |     |
| Beta-naphthol, 20%               | 100         | 100 | 100 | 100 | 100 | 100 | 100 | 100 | 100 | 100 |     |
| Beta-naphthol, 30%               |             |     |     |     |     |     |     |     |     |     |     |
| 10 "Cumar" AX                    |             |     |     |     | 30  |     | 100 | 100 | 67  | 102 | 100 |
| "Neville X-1"                    | 100         |     |     |     |     |     |     |     |     |     |     |
| Montan wax                       |             | 62  | 150 |     |     | 100 | 25  | 60  | 67  | 15  | 150 |
| FF wood rosin                    |             |     |     |     |     | 600 |     |     |     |     |     |
| G gum rosin                      | 407         | 608 | 682 |     |     |     |     | 433 | 402 |     |     |
| "Cumar" FX                       |             |     |     |     |     |     | 25  | 140 |     |     | 650 |
| Limed rosin (19° F.)             |             |     |     |     | 870 |     |     |     |     |     |     |
| 15 Black East India gum          |             |     |     |     |     |     | 200 |     |     |     |     |
| Temperature of plasticity (° C.) | 75          | 70  | 74  | 83  | 79  | 82  | 80  | 70  | 74  | 84  |     |
| Softening point (° C.)           | 85          | 81  | 77  | 95  | 85  | 89  | 87  | 77  | 76  | 92  |     |

| 20                               | Example No. |     |     |     |     |     |     |     |     |     | 20 |
|----------------------------------|-------------|-----|-----|-----|-----|-----|-----|-----|-----|-----|----|
|                                  | 67          | 68  | 69  | 70  | 71  | 72  | 73  | 74  | 75  |     |    |
| <b>Naphthol-modified rubber:</b> |             |     |     |     |     |     |     |     |     |     |    |
| Beta-naphthol, 10%               | 100         | 100 | 100 | 100 | 100 | 100 | 100 | 100 | 100 | 100 |    |
| Beta-naphthol, 20%               |             |     |     |     |     |     |     |     |     |     |    |
| Beta-naphthol, 30%               |             |     |     |     |     |     |     |     |     |     |    |
| 25 Montan wax                    | 60          | 100 | 66  | 50  | 162 | 100 | 100 | 60  | 100 |     |    |
| FF wood rosin                    | 240         | 360 | 400 | 525 | 648 | 800 | 600 | 240 | 800 |     |    |
| "Cumar" FX                       |             | 100 | 100 | 155 |     |     |     |     |     |     |    |
| Black East India gum             |             |     |     |     |     |     | 200 |     |     |     |    |
| Temperature of plasticity (° C.) | 83          | 75  | 74  | 70  | 73  | 71  | 80  | 74  | 72  |     |    |
| Softening point (° C.)           | 91          | 85  | 88  | 83  | 76  | 77  | 88  | 81  | 77  |     |    |

Table VI

| 35                                                  | Example No. |     | 35 |
|-----------------------------------------------------|-------------|-----|----|
|                                                     | 76          | 77  |    |
| <b>Naphthol-modified rubber: beta-naphthol, 20%</b> |             |     |    |
| "Cumar" AX                                          | 100         | 100 |    |
| Montan wax                                          | 27          | 20  |    |
| Paraffin                                            |             | 34  |    |
| FF wood rosin                                       | 7           | 14  |    |
| "Cumar" FX                                          |             | 330 |    |
| Temperature of plasticity (° C.)                    | 77          | 100 |    |
| Softening point (° C.)                              | 97          | 82  |    |

45 The following example illustrates the manner of using the impregnant compositions and the impregnated products of the invention:

Example 78.—A mixture of:

| 50          | Parts                                        |     | 50 |
|-------------|----------------------------------------------|-----|----|
|             | Naphthol-modified rubber (beta-naphthol 20%) | 100 |    |
| "Cumar" AX  |                                              | 15  |    |
| Montan wax  |                                              | 192 |    |
| G gum rosin | 461                                          |     |    |

55 is heated with stirring at 160–180° C. until homogeneous. This molten mixture is used to impregnate an 8 ounce/square yard wool-cotton felt by the dipping process. The impregnated sheet 60 is stripped at 0.039 inch between heated rods and then calendered to 0.050 inch and allowed to cool. Box toe blanks of the desired shape and size are stamped out of the sheet.

65 After skiving, a box toe blank is softened by being exposed to steam at 100° C. on the steamer for from 20 to 60 seconds and is then placed between the lining cloth and doubler cloth of the shoe upper and the whole assembly of leather, cloth, and box toe is pulled over on a pulling-over machine. The box toe blanks soften quickly on the steamer and become only slightly sticky. The box pulls over smooth and conforms to the last in the usual manner. When the shoe reaches the operation of bed-lasting the toe end 75 is inserted into a beehive steamer and the box

toe thereby softened again before bed-lasting. The box toe material remains soft for quick and easy lasting and conforms to the last, so that reheating and relasting are not necessary. The material is, however, capable of being reheated and relasted, if necessary.

No solvent is used in softening or lasting, but the lining adheres satisfactorily to the box toe. The inside of the lining is not stained.

It will be understood that all of the above examples are merely illustrative and that the invention broadly comprises, as a stiffener for shoes and the like, a web of fibrous material impregnated with an impregnant composed of beta-naphthol-modified rubber and an auxiliary component, the impregnant having a temperature of plasticity of 70–90° C. and a softening point of 75–100° C.

Instead of the wool-cotton felt used in Example 55, other webs of fibrous material may be used such as other varieties of felt, paper, flannel, canvas, duck, felted cellulose fiber such as that sold under the name "Krafelt", and the like.

It has been found that, when only one of the three classes of auxiliary ingredients is to be employed, the proportions should generally be, per 100 parts of beta naphthol-modified rubber, respectively: Of plasticizers, between 33 and 100 parts; of modifiers, between 13 and 18 parts; and of extenders, between 300 and 900 parts.

Where auxiliary ingredients of more than one of the three classes are used as a composite component of the impregnating composition, the range of operative mixtures cannot be expressed accurately in terms of limiting proportions of the three classes of auxiliary ingredients although the beta naphthol-modified rubber content of the impregnating composition should be not less than 10% and not more than 88%.

As indicated in the examples, coumarone indene resins of liquid or semi-liquid character have been found useful as plasticizers in the present impregnating compositions. These include Barrett Company's "Cumar AX" (melting range 75

20-30° C.) and "Cumar BX" (melting range 35-45° C.) and Neville Company's "Neville X-1". Montan wax is also a useful plasticizer but may be used in proportions up to 900 parts per 100 parts of beta naphthol-modified rubber, functioning as an extender in the higher proportions rather than a plasticizer.

5 Within the stated range of 33-100 parts for plasticizers the nature of the plasticizer selected will influence the specific amount used, that is, plasticizers having relatively lower melting points will be used generally in the lower part of the range of proportions given while the relatively higher melting point plasticizers will be used in 15 the higher part of the range of proportions given and, in fact, may even be used in excess of the upper limit of the proportion range.

10 The modifiers found useful in the present invention include paraffin wax (preferably of melting point of 50-59° C.), ceresin wax, and Japan wax.

15 Among the extenders suitable for use in the herein considered impregnating compositions may be mentioned gum rosin, wood rosin, and montan wax, all well adapted for use as the sole auxiliary ingredient in the composition, and Barrett Company's "Cumar FX" (melting range 125-130° C.), black East India gum, and limed rosin which are not particularly desirable as sole 20 auxiliary ingredients because they do not depress the softening temperature of the beta naphthol-modified rubber sufficiently.

25 The impregnating compositions of the present invention are readily formed by melting the ingredients together and, in molten condition, at temperatures low enough to cause no decomposition or degradation, are sufficiently mobile for the impregnation of fibrous webs by ordinarily available methods.

30 40 The impregnated webs made according to the present invention are readily blanked and skived by the usual methods and do not break down to dust.

45 Shoe stiffening members made in accordance with the invention, upon being placed in the steamer following the standard practice, become completely limp and soft, and sticky enough to adhere to the shoe lining but not so sticky as to adhere to the operator's fingers. The limpness is 50 retained, upon removal from the steamer, for a period entirely adequate to permit of the stretching of the piece over the last. The construction of the shoe may be carried out in the usual manner and at no stage during the wearing of the 55 shoe does the impregnant exert any staining or other deleterious effect upon the leather or fabric with which it is associated in the shoe.

60 Stiffening members made according to the present invention possess unusual rigidity and toughness in proportion to their thickness and, for this reason, are well adapted to provide adequate stiffening and support in a shoe without undesirable bulk. They do not deteriorate with age nor as a result of exposure, moisture, and perspiration incidental to hard wear. Also, they are water-proof in the ordinary sense of being undamaged by brief or prolonged immersion in water at ordinary temperatures.

65 70 As many apparently widely different embodiments of this invention may be made without departing from the spirit and scope thereof, it is

to be understood that the invention is not limited to the specific embodiments thereof except as defined in the appended claims.

We claim:

1. A stiffening member for shoes and the like, 5 comprising a web of fibrous material impregnated with a composition comprising essentially beta naphthol-modified rubber and a compatible auxiliary component from the group consisting of non-volatile, water-insoluble, organic plas- 10 ticizers, modifiers and extenders.

2. A stiffening member for shoes and the like, 15 comprising a web of fibrous material impregnated with a composition comprising essentially beta naphthol-modified rubber and a compatible auxiliary component from the group consisting of non-volatile, water-insoluble, organic plas- 20 ticizers, modifiers and extenders, said composition having a temperature of plasticity of 70-90° C. and a softening point of 75-100° C. 20

3. An impregnating composition for shoe stiff- 25 eners and the like comprising essentially beta naphthol-modified rubber and a compatible auxiliary component from the group consisting of non-volatile, water-insoluble, organic plas- 25 ticizers, modifiers, and extenders.

4. An impregnating composition for shoe stiff- 30 eners and the like comprising essentially beta naphthol-modified rubber and a compatible auxiliary component from the group consisting of non-volatile, water-insoluble, organic plas- 30 ticizers, modifiers, and extenders, said composi- 35 tion having a temperature of plasticity of 70-90° C. and a softening point of 75-100° C.

5. A stiffening member for shoes and the like, 35 comprising a web of fibrous material impregnated with a composition comprising 100 parts beta naphthol-modified rubber and 53-100 parts of coumarone indene resin, said resin having a melting range of from 20-45° C. 40

6. A stiffening member for shoes and the like, 45 comprising a web of fibrous material impregnated with a composition comprising 100 parts beta naphthol-modified rubber, 125-870 parts of rosin, and 20-147 parts of coumarone indene resin, said resin having a melting range of from 20-45° C.

7. A stiffening member for shoes and the like, 50 comprising a web of fibrous material impregnated with a composition comprising 100 parts beta naphthol-modified rubber, 50-800 parts montan wax, and 18-100 parts of coumarone indene resin, said resin having a melting range of from 20-45° C.

8. An impregnating composition for shoe stiff- 55 eners and the like comprising 100 parts beta naphthol-modified rubber and 53-100 parts of coumarone indene resin, said resin having a melt- 60 ing range of from 20-45° C.

9. An impregnating composition for shoe stiff- 65 eners and the like, comprising 100 parts beta naphthol-modified rubber, 125-870 parts of rosin, and 20-147 parts of coumarone indene resin, said resin having a melting range of from 20-45° C.

10. An impregnating composition for shoe stiff- 70 eners and the like, comprising 100 parts beta naphthol-modified rubber, 50-800 parts of montan wax, and 18-100 parts of coumarone indene resin, said resin having a melting range of from 20-45° C.

PAUL A. BALON. 70  
HAROLD S. HOLT.